

P. POETSCHKE.  
REINFORCED PAPER ARTICLE.  
APPLICATION FILED NOV. 5, 1917.

1,274,323.

Patented July 30, 1918.

*Fig. 1.*



*Fig. 2.*



*Fig. 3.*



Inventor  
Paul Poetschke

By *Oppenheimer Lawrence*,  
Attorneys

# UNITED STATES PATENT OFFICE.

PAUL POETSCHKE, OF MILFORD, DELAWARE.

## REINFORCED-PAPER ARTICLE.

1,274,323.

Specification of Letters Patent.

Patented July 30, 1918.

Application filed November 5, 1917. Serial No. 200,445.

To all whom it may concern:

Be it known that I, PAUL POETSCHKE, a citizen of the United States, residing at Milford, in the county of Sussex and State of Delaware, have invented certain new and useful Improvements in Reinforced-Paper Articles; and I do hereby declare the following to be a full, clear, and exact description of the invention, such as will enable others skilled in the art to which it appertains to make and use the same.

This invention relates to paper, and particularly to various shaped articles which may be made of paper, and has for one object, the provision of a container to receive articles of various natures, such for instance, as food products, chemicals and divers other substances, capable of being packed and marketed in metallic or glass containers or containers of various other materials, one of the objects of the present invention being to provide for the construction of containers of a material more rapidly and less expensively made, than possible when tin, glass, earthenware or other material is utilized.

Another object of the present invention is to improve the construction of paper, so that a paper of greater strength, rigidity, and durability is obtained, and which is waterproof by virtue of the materials of which it is constructed.

It is another object of the present invention to provide a paper which, while being waterproof by the introduction of a body of cementitious material between the surfaces of the sheet of paper, may also have applied to it on either or both of its surfaces applications of various materials as for instance, paraffin, rosin, shellac or any other suitable or appropriate water repellent which may be determined by the nature of the contents of the container in which the paper stock may be utilized.

The invention consists in an article of manufacture of paper, and embodiments of the article are illustrated in the accompanying drawing, in which,

Figure 1 is a perspective view of a container partly broken away to show the construction of the wall,

Fig. 2 is a perspective view of a sheet of the material partly broken away to show the construction, and

Fig. 3 is a detail perspective view of a fragment of a piece of the material Illus-

trating that embodiment of the invention employing exterior and interior coating.

It is desirable to substitute for various types of containers which are made of tin, glass, earthenware or other substances, containers of less expensive material and which will at the same time, have the desired properties of strength, durability, impermeability and rigidity not present in containers made of paper or fiber as now marketed, and which are impregnated with paraffin or other wax-like or appropriate substances, having the object of rendering the material more or less impervious to the material carried in the containers formed of the paper or fiber stock. Containers made of paper or fiber so impregnated are not only defective in the matter of durability and strength, but they also will gradually absorb the moisture of or be attacked by the contents of the container.

To overcome these various defects and provide a container or the like of paper or fiber stock of the desired strength and rigidity, and one which will also be impervious, my present invention contemplates the manufacture of an article, such, for instance as a container, by employing a suitable number of layers or sheets of paper, for instance, as illustrated at Fig. 1, in which 2 is an inner layer of paper or other suitable material to which is applied a mineral cementitious and preferably neutral cement 3, and outside of which there is another paper or other layer 4. Preferably the cement which I utilize is in the nature of an artificial stone and therefore, will inherently possess the desired characteristics of strength and rigidity, and water-proofing the article.

Also I utilize a cementitious material which has not only the desired water-proofing, and strengthening properties, but also is devoid of any agents which will be deleterious either to the material of which the container or article is manufactured, but also will not be harmful or injurious to the substances placed in the package or container, and one, which instead of becoming softened upon the application of heat, as glue, wax, paraffin and various other materials will, instead, harden at normal or increased temperatures.

As an example of the mineral, neutral, cementitious layer which may be introduced in the stock of which the container

is to be formed, I may employ magnesium oxid and silex in about equal proportion, which are mixed and reduced to plastic condition by the addition of a solution of magnesium chlorid of approximately 30 degrees Baumé. As above indicated, in the practice of the method of producing the article of whatever shape it may be, whether of sheet form or other shape, for instance, to produce a container, the plastic cement is introduced between the layers of the paper or fiber of which the article is to be made and with which any suitable number may be utilized. The sheet or shaped article built up by the above described method is allowed to harden when it is then ready for use. While the cementitious layer in the body of the article will harden at ordinary temperatures, I have found that a temperature of about 100 degrees Fahrenheit gives a very satisfactory result, the hardening taking place more rapidly than at lower temperatures, but for the purpose of more rapidly hardening the material, the article is subjected to a temperature approximately 350 degrees Fahrenheit, at which the cement will harden in about five minutes, the time varying of course, according to the thickness of the material, the shape of the article and the manner of the application of the heat.

This mineral cement is preferably applied as an intermediate or an intervening layer or body, so that when desired, the surfaces of the article may be coated with any other substance, such for instance, as rosin, shell-lac, paraffin or any mixtures thereof or other desired material, and as shown in Fig. 3, the inner and outer surfaces of the wall forming the container are indicated at 5 and 6, as being so coated, the nature of which will be determined by the use of the article, and it will be understood of course, that the interior and exterior coatings may be of different substances.

The article may be made of any number of layers of paper or fibrous material as indicated in Fig. 2 in which certain of the

layers are shown as perforated or of foraminous material as indicated at 7. In this form of the manufactured article, the cementitious material may be applied to both sides of the intermediate perforated layer or layers and will fill the interstices thereof, and in this way, greatly reinforce and strengthen the article. 50 55

The words "article of manufacture" are used in this specification and in the claims to refer to that product of whatever shape it may be which is constructed according to the steps of the method above defined and using materials having the properties herein set forth. 60

What is claimed is:

1. An article of manufacture comprising paper having a neutral, mineral, waterproofing reinforce consisting of magnesium oxid and silex mixed with magnesium chlorid. 65
2. An article of manufacture of paper having included therein a cementitious, mineral, reinforcing material, and an external application of waxy water-repellent. 70
3. An article of manufacture of paper having included therein a cementitious, mineral material, and having on its walls an application of waxy water-repellent. 75
4. An article of manufacture of paper reinforced by an included cement consisting of magnesium oxy-chlorid.
5. An article of manufacture composed of paper having an intermediate layer of magnesium oxid and silex reduced to plastic state by magnesium chlorid. 80
6. An article of manufacture composed of laminated, perforate and imperforate sheets with an associated body of cementitious material consisting of magnesium oxy-chlorid. 85
7. An article of manufacture of paper having included therein a cementitious, mineral material, and an external application of waxy resinous water-repellent. 90

In testimony whereof I affix my signature.

PAUL POETSCHKE.